

## [54] PROCESS FOR PRODUCING ENERGY IN A GAS GENERATOR SYSTEM

[75] Inventor: Donald Pilipovich, Ventura, Calif.

[73] Assignee: Rockwell International Corporation, El Segundo, Calif.

[22] Filed: Sept. 26, 1968

[21] Appl. No.: 762,938

[52] U.S. Cl. .... 60/218, 60/219, 149/109

[51] Int. Cl. .... C06d 5/04

[58] Field of Search..... 60/218; 149/109

## [56]

## References Cited

## UNITED STATES PATENTS

3,442,927 5/1969 Thompson et al. .... 149/109 X

Primary Examiner—Benjamin R. Padgett

Attorney—William R. Lane, Thomas S. MacDonald and Paul L. Sabatine

## [57]

## ABSTRACT

In a gas generator system, a process for producing hot gaseous power by heating bis-(fluoroformyl)-peroxide to give carbon dioxide, carbonyl fluoride, and oxygen.

4 Claims, 2 Drawing Figures



PATENTED JAN 8 1974

3,783,617



FIG. 1



FIG. 2

INVENTOR,  
DONALD PILIPOVICH

BY

*Paul L. Sabatine*

ATTORNEY

# PROCESS FOR PRODUCING ENERGY IN A GAS GENERATOR SYSTEM

## BACKGROUND OF THE INVENTION

This invention relates to a monopropellant gas generator. More specifically, the invention relates to the use of a chemical compound, bis-(fluoroformyl)-peroxide as a monopropellant gas generator.

The use of monopropellants as gas generators is well described in the prior art. Monopropellants are conventionally used in small rocket engines, for the attitude control of a space vehicle or in gas generators for rocket turbopump drives. The turbopump feed system in a rocket system is routinely driven by turbines that derive their power from the expansion of hot monopropellant gases. These latter gases are produced in a gas generator in the required quantities by means of chemical reaction of propellants similar to those in thrust chambers.

A monopropellant system must be chemically and thermally stable to insure good liquid storage properties, yet at the same time it must be easily decomposed and reactive to permit good combustion properties. The liquid type prior art monopropellants, hydrazine and hydrogen peroxide, are generally acceptable for certain, limited applications, but difficulties are often encountered in employing said monopropellants. For example, in a pressurizing tankage or expulsion system containing oxidizers the hydrazine cannot be used. Indeed, all presently known monopropellant gas generators are believed to present a hazardous situation when used to pressurize oxidizer propellant tankage.

The hazardous situation usually arises because of the incompatibility of the gas, formed from the monopropellant, and the oxidizer. For the purpose of illustration, the use of the monopropellant hydrazine  $N_2H_4$  as a pressurizing agent with the propellant oxidizer  $ClF_3$  is discussed immediately below. The hydrazine,  $N_2H_4$ , decomposes according to the following equation:  $N_2H_4 \rightarrow N_2 + 2H_2$ . While  $N_2$  is inert, the  $H_2$  decomposition product is also an excellent reducing agent and it will react vigorously with the oxidizer  $ClF_3$  according to the general equation  $ClF_3 + 2H_2 \rightarrow 3HF + HCl$ . Thus, the gases produced by the decomposition of the hydrazine are vigorously reactive with the oxidizer chlorine trifluoride and creates a hazardous condition. By producing unwanted hydrogen fluoride and hydrogen chloride in its application, condensable gases are formed which detract from the efficiency of operation.

The use of hydrogen peroxide as a monopropellant also produces undesirable conditions. For example, hydrogen peroxide decomposes to produce water and oxygen. The newly formed water reacts with oxidizers like chlorine trifluoride and chlorine pentafluoride to produce chlorine dioxide, a very sensitive and explosive material. The reactions between the monopropellant hydrogen peroxide and the oxidizer chlorine trifluoride can be represented by the following:  $2H_2O_2 \rightarrow 2H_2O + O_2$ ; and,  $3H_2O_2 + 2ClF_3 \rightarrow 2ClO_2 + 6HF + O_2$ . Thus, it will be readily appreciated by those versed in the subject art that a monopropellant gas must be chemically and thermally stable to insure good liquid storage properties and at the same time it must easily combust to permit good combustion and ignition properties. Because these requirements are essentially incompatible with most chemicals, there are relatively

few presently available monopropellants and even these have to be used carefully.

Accordingly, it is an object of this invention to provide an acceptable monopropellant gas.

Still a further object of the present invention is to provide a monopropellant gas generator system that does not produce reactive decomposition products.

Yet a further object of the present invention is to provide a gas generator that is compatible with oxidizers.

These objects, advantages and features will become readily apparent to those skilled in the art from the following specification and the appended claims.

## SUMMARY OF THE INVENTION

15 This invention is concerned with the use of a monopropellant gas generator, bis-(fluoroformyl)-peroxide,  $C_2F_2O_4$ . The compound decomposes on the application of heat to give  $COF_2$ ,  $CO_2$  and  $O_2$ .

The invention will further become better understood 20 by reference to the following detailed description of the accompanying drawing and disclosure. It is to be understood that the annexed sheet of drawing and disclosure is presented for the purpose of illustration of presently preferred embodiments of the present invention 25 and that the scope and spirit of the invention is not to be limited thereto.

## DESCRIPTION OF THE DRAWING

In accompanying drawing, FIG. 1, is shown a schematic view of an environment employing the inventive process disclosed herein, as a source of power in a turbopump system.

In accompanying drawing, FIG. 2, is set forth a schematic view of another novel embodiment of the invention in a generalized pressure fed system.

## DESCRIPTION OF THE INVENTION

In attaining the object and features of the present invention, it has now been unexpectedly found that bis-(fluoroformyl)-peroxide,  $C_2F_2O_4$ , can be successfully employed as a monopropellant.

The compound bis-(fluoroformyl)-peroxide, can be easily formed by intimately reacting  $O_2$ ,  $CO$  and  $F$  at a temperature between  $0^\circ C$  and  $50^\circ C$ . The product of the reaction is a clear liquid,  $C_2F_2O_4$ . The chemical equation for this reaction can be represented by the equation



The compound has a boiling point of  $15.9^\circ C$  and it crystallizes into a white mass at  $-43^\circ C$ . The compound can also be prepared according to the procedure as set forth by A. J. Arvia, et al., *Quim. Arg.*, Vol. 50, p. 135-143, 1962 and in *Chemical Abstracts*, Vol. 54, p. 16384 h, 1960.

Bis-(fluoroformyl)-peroxide is chemically and physically suited as a gas generator because it readily decomposes at  $100^\circ C$  and above to give  $CO_2$ ,  $COF_2$  and  $O_2$  in a mol ratio of 1:1:0.5. The chemical decomposition can be represented by the equation



$COF_2 + CO_2 + \frac{1}{2}O_2$ . The products formed by the decomposition of bis-(fluoroformyl)-peroxide,  $CO_2$ ,  $COF_2$  and  $O_2$  are quite compatible with halogen fluo-

rides such as chlorine trifluoride, bromine pentafluoride, chlorine pentafluoride and the like, and with oxygen oxidizers such as dinitrogen tetroxide and the like at elevated temperatures. In addition, the decomposition reaction products of bis-(fluoroformyl)-peroxide are non-explosive, non-catastrophic and can be contained in non-specific tankage housing. Accordingly, it will be readily seen to those skilled in the present art that bis-(fluoroformyl)-peroxide is ideally suited as a monopropellant gas generator.

An embodiment of this invention as set forth in FIG. 1, consists of a gas generator 10, provided with a suitable heating means 11, such as an induction heating coil or like device, connected to a power source 13, such as a battery or the like. A conduit 14 is connected between gas generator 10 and turbopump 12, to provide power to turbine blade 20 for operating oxidizer pump 16 and fuel pump 18. Turbopump assembly 12 comprises an oxidizer pump 16 and fuel pump 18, with turbine blade 20 therebetween. The oxidizer pump 16 is fed from oxidizer tank 22 with suitable exit means 26 to a combustion chamber (not shown) and fuel pump 18 is fed from fuel tank 24 with suitable exit means 28 to the aforementioned combustion chamber.

Turning now to the accompanying drawing, FIG. 1; 25 in operation, said gas generator is charged with bis-(fluoroformyl)-peroxide and selectively heated to 100°C or above to produce the non-reactive and non-corrosive gases as described above, COF<sub>2</sub>, CO<sub>2</sub> and O<sub>2</sub>. The gases formed as a result of thermal decomposition are next conveyed through the conduit 14 to turn the turboblade 20 which in turn provides the necessary power to operate pump 16 and 18 for conveying the oxidizer and fuel to the combustion chamber for powering the rocket engine. Thus, it can be seen, that the 30 monopropellant gas generator of this invention can be used in a gaspressurized generator system or the like, or in a system similar to a conventional gas pressurized rocket system. The gases produced on heating the monopropellant to its gaseous decomposition point are fed in by manifold or pipe to the turbine or the like and are there expanded in the turbine nozzle to run the turbine. The monopropellant gas generator of this invention can be entirely self-starting and it does not require any special starting provisions or catalytic decomposition agents.

Referring now to accompanying drawing, FIG. 2; in operation, is a general pressure fed propellant system wherein the monopropellant bis-(fluoroformyl)-peroxide in tank 34 is pressurized by means of a small 5 amount of a suitable gas such as nitrogen or the like stored in tank 30 through a pressure regulator 32. The monopropellant is conveyed from tank 34 through suitable means, such as a conduit, pipe or the like, into an injector 36 which feeds the monopropellant into a thermal initiation unit 38 wherein the monopropellant thermally decomposes to produce COF<sub>2</sub>, CO<sub>2</sub> and O<sub>2</sub>. The newly formed gases are then fed from unit 38 into propellant tank 40 which contains chlorine trifluoride or other like agents, and forces said agent under pressure 10 through a suitable conduit into thrust chamber 42. While schematic drawing FIG. 2 depicts a single propellant ullage flow system, it is to be understood that in actual practice a bipropellant system, mixing for example, methyl hydrazine and chlorine trifluoride, would be employed. In a bipropellant system a single gas generator interconnected to two tanks similar to tank 40 could be employed, or two independent gas generator systems having their own ullage flow may be used for feeding oxidizers and fuels into a thrust chamber.

Obviously, many modifications and variations of the instant invention are possible in the light of the above teachings, and it is, therefore, to be understood that within the scope of the claims, the invention may be practiced otherwise as specifically described.

I claim:

1. The process comprising thermally decomposing bis-(fluoroformyl)-peroxide at a temperature above about 100°C to produce a gaseous product consisting essentially of oxygen, carbon dioxide and carbonyl fluoride in a mol ratio of about 0.5:1:1 and using said gaseous product as a source of power.
2. The process of claim 1 in which the gaseous product is used as a source of power to drive a turbine.
3. The process of claim 1 in which the gaseous product is used as a source of power for conveying a fuel into a rocket thrust chamber.
4. The process of claim 1 in which the gaseous product is used as a source of power for conveying an oxidizer into a rocket thrust chamber.

\* \* \* \* \*